

# United States Patent Office

2,938,871

Patented May 31, 1960

1

2,938,871

## AVIATION GAS TURBINE LUBRICANTS

Alfred H. Matuszak, Westfield, Ernest V. Wilson, Cranford, and Walter W. Gleason, Roselle, N.J., assignors to Esso Research and Engineering Company, a corporation of Delaware

No Drawing. Filed Dec. 24, 1956, Ser. No. 630,060

4 Claims. (Cl. 252—49.9)

This invention relates to synthetic lubricating compositions. Particularly, the invention relates to lubricating compositions comprising a synthetic ester lubricating oil and minor amounts of certain additives which improve the load-carrying ability of the synthetic oil.

Synthetic ester lubricating oils are known to the art. In general, these oils are characterized by viscosity properties that are outstanding at both low and high temperatures, especially when compared to mineral oils. In recent years, the synthetic ester oils have become of increasing importance in the field of lubrication, and one of the most important current applications of such compounds is in the lubrication of aviation gas-turbine systems such as are used in the "turbo-jet" or "turbo-prop" type of aircraft. However, in general, the load-carrying ability of these ester oils is not particularly high. Because of the increasing severity of the conditions prevailing in the lubrication of aviation gas-turbine systems, it is highly desirable to form synthetic ester lubricating compositions having higher load-carrying ability than is inherent in the ester oil itself. This invention, therefore, is concerned with synthetic ester oils containing additives for increasing the load-carrying ability of the oil.

In general, the compositions of this invention will comprise a synthetic ester lubricating oil and minor load-carrying improving amounts of saturated aliphatic dicarboxylic acids containing 6 to 10 carbon atoms per molecule. Although these dicarboxylic acids are very effective as load-carrying agents, the amount in which they can be used is limited, since they are not generally soluble in ester oils in amounts greater than 0.10% by weight. It has also been found that small amounts of aryl phosphate and halogen-substituted alkyl phosphorus compounds are also very effective in increasing the load-carrying ability of the ester lubricant. Surprisingly, it has been further found that the combination of the dicarboxylic acid with small amounts of (a) the halogen-substituted alkyl phosphorus compound, or (b) a mixture of both the aryl phosphate and the halogen-substituted alkyl phosphorus compounds, results in an additive combination having a much greater effect on the load-carrying ability of the synthetic ester lubricant than would be expected from the mere addition of the individual effect of each component.

The ester oils used in the compositions of this invention include diesters of saturated aliphatic dicarboxylic acids esterified with alcohols. These diesters have the general formula:



wherein R represents a straight-chain or branched-chain alkyl radical of an alkanol having about 7 to 13 carbon atoms, R<sub>1</sub> is a straight or branched-chain C<sub>4</sub> to C<sub>8</sub> alkylene radical of a dicarboxylic acid, and the total number of carbon atoms in the molecule being about 20 to 36, preferably 22 to 26. Examples of such diesters in-

2

clude di-2-ethylhexyl sebacate, di-n-nonyl adipate, di-n-tridecyl azelate, di-n-heptyl isosebacate, di-C<sub>8</sub> Oxo trimethyl adipate, di-C<sub>13</sub> Oxo pimelate, etc. The diesters prepared from the Oxo alcohols, which are isomeric mixtures of highly branched-chain aliphatic primary alcohols, are particularly desirable. The Oxo alcohols have a very high degree of branching in the hydrocarbon chain, which results in diester oils having low pour points and low viscosity at low temperature. These alcohols are prepared from olefins, such as polymers and copolymers of C<sub>3</sub> and C<sub>4</sub> monoolefins, which are reacted with carbon monoxide and hydrogen, in the presence of a cobalt-containing catalyst such as a cobalt carbonyl catalyst, at temperatures of about 300° to 400° F., and under pressures of about 1000 to 3000 p.s.i., to form aldehydes. The resulting aldehyde product is then hydrogenated to form the alcohol which is then recovered from the hydrogenation product.

The dicarboxylic acids which may be used as load-carrying agents are those saturated aliphatic dicarboxylic acids having 6 to 10 carbon atoms per molecule. These acids include adipic acid, pimelic acid, suberic acid, azelaic acid, sebacic acid and isosebacic acid. The isosebacic acid is a mixture of C<sub>10</sub> acids comprising about 60 to 90 wt. percent of  $\alpha$ -ethyl suberic acid, about 5 to 25 wt. percent of  $\alpha, \alpha'$ -diethyl adipic acid, and about 5 to 15 wt. percent of sebacic acid. A typical such acid will contain about 75 wt. percent of  $\alpha$ -ethyl suberic acid, about 15 wt. percent of  $\alpha, \alpha'$ -diethyl adipic acid and about 10 wt. percent of sebacic acid.

The aryl phosphates useful in this invention are those compounds which have the following general formula:

35



40

wherein each R is a radical selected from the group consisting of hydrogen and alkyl groups containing about 1 to 4 carbon atoms, e.g. methyl groups. Examples of such phosphates include triphenyl phosphate, phenyl di-cresylphosphate, tricresylphosphate, methyl di-tert. butyl phosphate, etc.

The halogen-substituted alkyl phosphorus compounds useful in this invention may be divided into three general classes as follows:

45

50 Halogen (e.g. chlorine) phosphonates which include saturated and unsaturated, mono, di and tri halogen-substituted alkyl phosphonates having the general formula:

55



60

wherein R, R' and R'' are aliphatic hydrocarbon radicals or halogen-substituted aliphatic hydrocarbon radicals, said radicals containing 1 to 5, e.g. 2 to 4, carbon atoms and at least one of said radicals is halogen-substituted. For example, R may be a halogen-substituted alkyl radical, R' may be either an alkyl radical or a

65

halogen-substituted alkyl radical and R'' may be an alkylene radical of from 2 to 5 carbon atoms. Specific examples of compounds which may be used include mono beta chloroethyl, monoethyl, vinyl phosphonate; bis(beta chloroethyl) vinyl phosphonate; bis(beta chloroethyl) beta chloroethyl phosphonate; bis(beta chloroethyl) ethyl phosphonate; bis(4-chloropentyl) butylene

phosphonate; mono(3-chloropentyl)butyl-1, propyl phosphonate; etc.

Halogen phosphites having the general formula:



wherein R represents a halogen-substituted alkyl group containing about 1 to 5, e.g. 2 to 4, carbon atoms and each R' contains 1 to 5, e.g. 2 to 4 carbon atoms and is either an alkyl radical or a halogen-substituted alkyl radical.

Halogen phosphates having the general formula:



wherein R represents a halogen-substituted alkyl group containing about 1 to 5, e.g. 2 to 4, carbon atoms, and each R' contains 1 to 5, e.g. 2 to 4, carbon atoms and is either an alkyl group or a halogen-substituted alkyl group.

The lubricating composition of the invention will comprise a major proportion of a synthetic ester lubricating oil containing a load-carrying improving amount of the additives of the invention. The oil will contain about 0.01 to 0.1 wt. percent, e.g. 0.04 to 0.06 wt. percent of a saturated aliphatic dicarboxylic acid having 6 to 10 carbon atoms and may also contain about 0.5 to 5.0 wt. percent, e.g. 1.0 to 3.0 wt. percent of an aryl phosphate and/or about 0.1 to 0.8 wt. percent, e.g. 0.4 to 0.5 wt. percent of a halogen-substituted alkyl phosphorus compound, said wt. percent being based on the amount of oil.

Other lubricating oils may also be incorporated into the above composition. For example, mineral oil or other synthetic oils, such as complex ester oils may be added. Other additives may also be added, including oxidation inhibitors such as phenothiazine, phenyl  $\alpha$ -naphthylamine, rust preventive additives, such as petroleum sulfonates, lecithin, Span 80; viscosity index improvers, such as polymethacrylates, polyethylene; etc. Greases may also be prepared by thickening the lubricating oil composition of this invention with appropriate grease thickeners.

The invention will be further understood by the following examples which include preferred embodiments of the invention.

#### EXAMPLE I

1.0 wt. percent (based on the weight of oil) of tricresyl phosphate was added to a base oil consisting of a synthetic diester oil containing 1.0 wt. percent of phenothiazine as an oxidation inhibitor. The synthetic diester oil was a mixture of 50 vol. percent of a di-C<sub>8</sub> Oxo adipate and 50 vol. percent of a di-C<sub>10</sub> Oxo adipate. The C<sub>8</sub> alcohol used in preparing the adipate was prepared by subjecting butylene-propylene copolymers having 7 carbon atoms to the Oxo process. The C<sub>10</sub> alcohol used in preparing the C<sub>10</sub> adipate was a similar type alcohol prepared by subjecting tripropylene to the Oxo process.

The above blend was then tested for load-carrying ability in a Standard MIL-L-7808C Ryder Gear Test, which test is known in the art.

#### EXAMPLES II TO IX

Various blends of additives were prepared in the same ester oil base of Example I, and were tested for their load-carrying ability. The results of these tests and the compositions used are given in the following table.

| 5  | Example No.     | Additive in Ester Oil <sup>1</sup> (Wt. Percent Based on Weight of Base) |              |                                              | Ryder Gear Test (Load Carried in Pounds/Inch) |
|----|-----------------|--------------------------------------------------------------------------|--------------|----------------------------------------------|-----------------------------------------------|
|    |                 | Tri-cresyl Phosphate                                                     | Sebacic Acid | Bis( $\beta$ -chloroethyl) vinyl phosphonate |                                               |
| 10 | Base            |                                                                          |              |                                              | 1,750                                         |
|    | I               | 1.0                                                                      |              |                                              | 1,860                                         |
|    | II <sup>2</sup> |                                                                          | 0.050        |                                              | 1,990                                         |
|    | III             |                                                                          | 0.100        |                                              | 2,150                                         |
|    | IV              |                                                                          |              | 0.50                                         | 2,350                                         |
|    | V               | 1.0                                                                      | 0.050        |                                              | 2,100                                         |
|    | VI              | 1.0                                                                      | 0.10         |                                              | 2,160                                         |
|    | VII             | 1.0                                                                      |              | 0.50                                         | 2,370                                         |
| 15 | VIII            |                                                                          | 0.05         | 0.50                                         | 2,920                                         |
|    | IX              | 1.0                                                                      | 0.05         | 0.50                                         | 3,870                                         |

<sup>1</sup> The base was an ester oil which consisted of 50 vol. percent C<sub>8</sub> Oxo adipate and 50 vol. percent C<sub>10</sub> Oxo adipate and containing 1 wt. percent phenothiazine.

<sup>2</sup> This blend also contained 1 wt. percent of a complex ester formed from 2 moles of C<sub>8</sub> Oxo alcohol, 2 moles of adipic acid and 1 mole of polyethylene glycol (200). However, this proportion of complex ester had an insignificant effect on the Ryder Gear Test.

<sup>3</sup> Replacing the 0.05% sebacic acid with 0.05% isosebacic acid resulted in 1970 lb./inch load.

As seen from the above table, the ester oil (base) carried 1750 pounds. The addition of 1.0 wt. percent of tricresyl phosphate (Example I) increased the Ryder Test value to 1860. The 1.0 wt. percent tricresyl phosphate therefore contributes about 110 lbs. of load-carrying ability. Sebacic acid (Examples II and III), when used in very small amounts, increased the load carried in about proportion to the sebacic acid concentration. The base oil plus 0.05% sebacic acid carried 1990 lbs., the sebacic acid contributing 240 lbs. Bis( $\beta$ -chloroethyl) vinyl phosphonate was also effective by itself (Example IV). The base oil plus 0.5% of this additive carried 2350 lbs., which shows the bis( $\beta$ -chloroethyl) vinyl phosphonate contributes 600 lbs. to the load. While the values obtained for Examples V, VI and VII were only about what would be calculated or expected by adding the individual effect of each component above, the results of Examples VIII and IX, as shown in the following table, were far greater than would be calculated by combining the effect of each additive component. Example VIII had a Ryder Test result of 2920 pounds. This is 330 lbs. more than the 2590 lbs. load that would be expected by adding the individual effects of the 0.05% sebacic acid and the 0.5% bis( $\beta$ -chloroethyl) vinyl phosphonate to the 1750 lbs. load carried by the base oil alone. Example IX, which is the same as Example VIII plus 1.0% tricresyl phosphate, carried a load of 3870 lbs. This is 1170 lbs. more than the 2700 lbs. load that would be calculated from the three additive components. In each of these two examples, synergism is clearly demonstrated. These results are summarized in the following table.

Table II

|      |                                                                                 | Ryder Gear Load, lbs./inch |        |
|------|---------------------------------------------------------------------------------|----------------------------|--------|
|      |                                                                                 | Calculated                 | Actual |
| 60   | Base                                                                            |                            | 1,750  |
| V    | Base+1% tricresyl phosphate+0.05% sebacic acid                                  | 2,100                      | 2,100  |
| 65   | VI                                                                              | 2,260                      | 2,180  |
| VII  | Base+1.0% tricresyl phosphate+0.10% sebacic acid                                | 2,360                      | 2,370  |
| VIII | Base+1.0% tricresyl phosphate+0.5% bis( $\beta$ -chloroethyl) vinyl phosphonate | 2,500                      | 2,920  |
| 70   | IX                                                                              | 2,700                      | 3,870  |

Examples of other compositions (in parts by weight) embraced within the purview of this invention are given in the following table.

|                                      | Composition of Lubricant (Parts) |      |     |      |      |      |      |
|--------------------------------------|----------------------------------|------|-----|------|------|------|------|
|                                      | A                                | B    | C   | D    | E    | F    | G    |
| Diester Oil:                         |                                  |      |     |      |      |      |      |
| Di-2-ethylhexyl sebacate             | 55                               | 70   |     | 30   | 100  |      | 40   |
| C <sub>8</sub> Oxo Azelate           |                                  |      | 50  | 40   |      | 100  | 40   |
| C <sub>10</sub> Oxo Adipate          | 45                               |      | 50  | 10   |      |      | 10   |
| C <sub>12</sub> Oxo adipate          |                                  | 30   |     | 20   |      |      | 10   |
| Dibasic Acid:                        |                                  |      |     |      |      |      |      |
| Iso-sebacic acid                     |                                  |      | 0.1 | 0.05 |      |      |      |
| Azelaic acid                         | 0.05                             |      |     |      | 0.05 | 0.05 | 0.05 |
| Adipic Acid                          |                                  | 0.05 |     | 0.05 |      |      |      |
| Aryl Phosphate:                      |                                  |      |     |      |      |      |      |
| Triphenyl phosphate                  |                                  | 1.0  |     | 1.0  |      |      |      |
| Phenyl diresyl-phosphate             | 3.0                              |      |     | 1.0  |      |      | 1.0  |
| Halo-Phosphorus Compound:            |                                  |      |     |      |      |      |      |
| Methyl di-tert. butyl phosphate      |                                  |      | 1.0 |      |      |      |      |
| Tris(2-chloroethyl) phosphate        |                                  |      |     |      |      |      |      |
| Bis(2-chloroethyl) vinyl phosphonate | 0.3                              |      |     |      | 0.2  |      |      |
| Bis(2-chloroethyl) ethyl phosphonate |                                  | 0.5  |     | 0.5  |      |      |      |
| Tris(2-chloroethyl) phosphite        | 0.3                              |      |     |      | 0.3  | 0.1  |      |
| Other additives:                     |                                  |      |     |      |      |      |      |
| Phenothiazine                        | 1                                |      | 1   |      | 1    | 1    |      |
| Phenyl alpha naphthylamine           |                                  | 1    |     | 1    |      |      | 1    |

What is claimed is:

1. A synthetic ester lubricating oil composition having improved load-carrying ability, which comprises a major proportion of a diester having the formula



wherein R represents an alkyl radical of an alkanol having about 7 to 13 carbon atoms, R<sub>1</sub> is a C<sub>4</sub> to C<sub>8</sub> alkylene radical of a dicarboxylic acid, and the total number of carbon atoms in the molecule being about 20 to 36; and about 0.01 to 0.10 wt. percent, based on the amount of diester, of a saturated aliphatic dicarboxylic acid containing about 6 to 10 carbon atoms per molecule and about 0.01 to 1.0 wt. percent of a halogen-containing phosphonate having the general formula:



wherein R, R' and R'' are selected from the group consisting of aliphatic hydrocarbon radicals and halogen-substituted aliphatic hydrocarbon radicals, each of said radicals containing 1 to 5 carbon atoms and at least one of said radicals being halogen-substituted.

2. A composition according to claim 1 wherein said dicarboxylic acid is sebacic acid and wherein said halogen-containing phosphonate is bis(β-chloroethyl) vinyl phosphonate.

5 3. A synthetic ester lubricating oil composition having improved load-carrying ability, consisting essentially of a diester having the formula ROOC-R<sub>1</sub>-COOR where-  
in R represents an alkyl radical of an alcohol having about 7 to 13 carbon atoms, R<sub>1</sub> is a C<sub>4</sub> to C<sub>8</sub> alkylene radical of a dicarboxylic acid, and the total number of carbon atoms in the molecule being about 20 to 36; about 0.01 to 0.10 wt. percent of a saturated aliphatic dicarboxylic acid containing about 6 to 10 carbon atoms per molecule, about 0.5 to 5.0 wt. percent of an aryl phosphate having the general formula:



15 wherein each R is a radical selected from the group consisting of hydrogen and alkyl groups containing about 1 to 5 carbon atoms; and about 0.1 to 0.8 wt. percent of a halogen-containing phosphonate having the general formula:



20 30 wherein R, R' and R'' are selected from the group con-  
sisting of aliphatic hydrocarbon radicals and halogen-  
substituted aliphatic hydrocarbon radicals, said radicals  
containing 1 to 5 carbon atoms and at least one of said  
radicals being halogen-substituted.

35 35 4. A composition according to claim 3 wherein said dicarboxylic acid is sebacic acid; said aryl phosphate is tricresyl phosphate; and wherein said phosphonate is bis(β-chloroethyl) vinyl phosphate.

#### References Cited in the file of this patent

#### UNITED STATES PATENTS

- 2,573,568 Harman et al. Oct. 30, 1951  
2,767,142 Morris et al. Oct. 16, 1956  
2,788,326 Bondi Apr. 9, 1957

#### FOREIGN PATENTS

- 744,777 Great Britain Feb. 15, 1956  
757,023 Great Britain Sept. 12, 1956

#### OTHER REFERENCES

- "Lubrication Engineering," August 1952, pages 177-179, 197-200.